# EUROPEAN PATENT SPECIFICATION

(11) **EP 4 353 803 B1**
(45) Date of publication and mention of the grant of the patent: **30.07.2025**
(21) Application number: 22210049.7
(22) Date of filing: 28.11.2022
(51) Int. Cl.: C10M 105/38, C10M 171/00

(54) **BASE OIL COMPRISING POLYOL ESTER AND REFRIGERATING MACHINE OIL COMPOSITION COMPRISING THE SAME**
BASISÖL MIT POLYOLESTER UND KÜHLMASCHINENÖLZUSAMMENSETZUNG DAMIT
HUILE DE BASE COMPRENANT UN ESTER DE POLYOL ET COMPOSITION D'HUILE POUR MACHINE FRIGORIFIQUE COMPRENANT CELLE-CI

(30) Priority: 13.10.2022 KR 20220131570
(43) Date of publication of application: 17.04.2024
(73) Proprietor: GS Caltex Corporation, Seoul 06141 (KR); Aekyung Chemical Co., Ltd., Seoul 04051 (KR)
(72) Inventor: BAEK, Joo-Young, 34122 Daejeon (KR); YOON, Eui-Jung, 34122 Daejeon (KR); SONG, Jae-Wook, 34108 Daejeon (KR); OH, Sung-Ho, 34108 Daejeon (KR); SEO, Ji-Hwan, 34108 Daejeon (KR)
(74) Representative: Zacco Sweden AB

(56) References cited:
- CN-A- 104 087 390
- US-A- 5 906 769
- US-A1- 2016 281 017

## Description

### BACKGROUND

### Field

The present disclosure relates to a refrigerating machine oil composition comprising polyol ester (POE). More specifically, the present disclosure relates to a refrigerating machine oil composition comprising polyol ester having excellent miscibility with polar refrigerant among refrigerants for a refrigerating machine as a base oil, and having excellent chemical stability.

### Related art

A compression-type refrigerating machine is a refrigeration system equipped with at least a compressor, a condenser, an expansion mechanism (such as an expansion valve), and an evaporator. Refrigerant and a refrigerating machine oil composition are mixed with each other and circulated within a sealed refrigeration system. Further, in the compression-type refrigerating machine, high and low temperature environments are created according to a compression ratio and phase change. Thus, a mixture of the refrigerant and the refrigerating machine oil composition is required to circulate in the refrigeration system without undesired phase separation even within a wide temperature range from low to high temperatures.

Conventionally, chlorofluorocarbon (CFC), hydrochlorofluorocarbon (HCFC), etc. have been mainly used as refrigerants for the refrigerating machine. However, CFC and HCFC are compounds comprising chlorine that causes environmental problems (destruction of the ozone layer). Thus, alternative refrigerants that do not contain chlorine such as hydrofluorocarbon (HFC) have been considered.

For example, 1,1,1,2-tetrafluoroethane, a 5:5 mixture of 1,1,1,2-tetrafluoroethane and pentafluoroethane, pentafluoroethane, and trifluoromethane (hereinafter, referred to as R134a, R410A, R125, and R23, respectively) as the hydrofluorocarbon (HFC) have attracted attention. For example, R134a has been used for the refrigerator system, and R410A has been used for an air conditioning system.

However, there was a concern that the HFC-based refrigerant may also have an adverse effect on global warming. Accordingly, as a so-called eco-friendly refrigerant that has a lower effect on ozone layer depletion and is more suitable for environmental protection, a refrigerant having a relatively low global warming potential (GWP) is attracting attention. The eco-friendly refrigerant includes, for example, difluoromethane (hereinafter, referred to as R32) as an HFC-based refrigerant; 2,3,3,3-tetrafluoro-1-propene(hereinafter, referred to as R1234yf) as an HFO-based refrigerant comprising olefin bonds; and a mixture of R32 and R1234yf at 68.9: 31.1 and a mixture of R1234yf and R134a at 56: 44 (hereinafter, referred to as R454B and R513A, respectively) as mixed refrigerant of HFC and HFO; and isobutane and propane (hereinafter referred to as R600a and R290, respectively) as a HC-based refrigerant composed of hydrocarbons.

US2016281017A1 shows a refrigeration oil comprising polyol ester and a refrigeration lubricant composition comprising the refrigeration oil and R32. CN104087390A shows a refrigerating machine oil comprising: an antioxidant, an anticorrosive agent, an antiwear agent, an antifoaming agent, with a balance of polyol ester. US5906769A shows a lubricant for use in air conditioner and refrigerator compressors, the lubricant comprising mixed esters of hindered polyols, most desirably di-pentaerythritol, usually mixed with some pentaerythritol, with a mixture of carboxylic acids including at least some of each of iso-pentanoic acid and iso-nonanoic acid.

Therefore, it is necessary to develop a base oil having excellent miscibility (compatibility) with various refrigerants, especially, refrigerants with high polarity, and at the same time, having high chemical resistance and abrasion resistance and excellent chemical stability when used in the refrigerating machine. Further, it is necessary to develop a refrigerating machine oil composition comprising the same.

### SUMMARY

### Technical purpose

A purpose of the present disclosure is to provide a base oil comprising a polyol ester having excellent miscibility with highly polar refrigerants, especially eco-friendly refrigerants with high polarity and low global warming potential (GWP), and having high abrasion resistance through relatively high viscosity.

Another purpose of the present disclosure is to provide a refrigerating machine oil composition that contains the base oil comprising polyol ester, and has excellent chemical stability.

Purposes of the present disclosure are not limited to the above-mentioned purpose. Other purposes and advantages of the present disclosure that are not mentioned may be understood based on following descriptions, and may be more clearly understood based on embodiments of the present disclosure. Further, it will be easily understood that the purposes and advantages of the present disclosure may be realized using means shown in the claims and combinations thereof.

### Technical purpose

One aspect of the present disclosure may provide a refrigerating machine oil composition comprising: a base oil comprising polyol ester, wherein the polyol ester is synthesized using: a polyhydric alcohol containing 5 or more hydroxyl groups; a first fatty acid as a linear fatty acid having 4 to 6 carbon atoms; a second fatty acid as a branched fatty acid having 4 to 6 carbon atoms; and a third fatty acid as a linear or branched fatty acid having 7 to 10 carbon atoms, wherein in synthesizing the polyol ester, a sum of a content of the first fatty acid and a content of the second fatty acid is in a range of 50 to 80 wt%, and a content of the third fatty acid is in a range of 20 to 50 wt%, based on 100 wt% of a total weight of the first fatty acid, the second fatty acid, and the third fatty acid, wherein the polyol ester has a kinematic viscosity at 40°C (KV40) in a range of 95 to 105 cSt, wherein the refrigerating machine oil further comprises at least one additive selected from a group consisting of a corrosion inhibitor and an acid scavenger, whereby both a corrosion inhibitor and an acid scavenger are present, wherein the refrigerating machine oil composition has a kinematic viscosity at 40°C (KV40) in a range of 70 to 90 cSt, wherein a total acid number (TAN) of the refrigerating machine oil composition is in a range of 0.010 to 0.100 mgKOH/g, wherein when a total weight of the refrigerating machine oil composition is 100 wt%, a content of the corrosion inhibitor is in a range of 0.03 to 0.10 wt%, and a content of the acid scavenger is in a range of 0.50 to 3.00 wt%, wherein the polyol ester has a floc point of -30°C or lower as measured according to following measurement method (1):
[Measuring method (1)] The floc point is measured according to ASHRAE STANDARD 86, based on a content of 80 vol% of a refrigerant used with the polyol ester and having a global warming potential (GWP) of 0 to 2,500, based on a total of 100 vol% of the polyol ester and the refrigerant,
wherein the refrigerating machine oil composition satisfies a following condition (A): $1 \left(TAN\right) f - \left(TAN\right) i 1 \leq 0.03$
where (TAN)i means a TAN value measured immediately after preparation of the refrigerating machine oil composition, and (TAN)f means a TAN value measured after aging of the refrigerating machine oil composition according to ASHRAE STANDARD 97.

In one embodiment, the refrigerant may include at least one selected from a group consisting of R32, R410A, R134a, R1234yf, R454B and R513A.

In one embodiment, when a total weight of the first fatty acid and the second fatty acid is 100 wt%, a content of the first fatty acid may be in a range of 30 to 50 wt%, and a content of the second fatty acid may be in a range of 50 to 70 wt%.

In one embodiment, the polyhydric alcohol may include dipentaerythritol.

In one embodiment, the corrosion inhibitor may include a benzotriazole-based compound.

In one embodiment, the acid scavenger may include a glycidyl ether-based compound.

In one embodiment, the refrigerating machine oil composition may further comprise at least one additive selected from a group consisting of an antioxidant and a wear resistance enhancer.

In one embodiment, the refrigerating machine oil composition may be used in at least one selected from a group consisting of an air conditioner, a refrigerator, and an air conditioner for a vehicle.

### Technical effect

The base oil comprising the polyol ester according to the present disclosure may have an excellent miscibility with a refrigerant having polarity and having low global warming potential (GWP).

The base oil comprising the polyol ester according to the present disclosure may have a high viscosity.

The refrigerating machine oil composition containing the base oil comprising the polyol ester according to the present disclosure may have significantly improved chemical stability.

In addition to the above-described effects, the specific effects of the present disclosure will be described together while describing specific details for following the invention.

### DETAILED DESCRIPTIONS

Advantages and features of the present disclosure, and a method of achieving the advantages and features will become apparent with reference to embodiments described later in detail together with the accompanying drawings. However, the present disclosure is not limited to embodiments as disclosed below, but may be implemented in various different forms. Thus, these embodiments are set forth only to make the present disclosure complete, and to completely inform the scope of the present disclosure to those of ordinary skill in the technical field to which the present disclosure belongs, and the present disclosure is only defined by the scope of the claims.

Further, descriptions and details of well-known steps and elements are omitted for simplicity of the description. Furthermore, in the following detailed description of the present disclosure, numerous specific details are set forth in order to provide a thorough understanding of the present disclosure. However, it will be understood that the present disclosure may be practiced without these specific details. In other instances, well-known methods, procedures, components, and circuits have not been described in detail so as not to unnecessarily obscure aspects of the present disclosure.

The terminology used herein is directed to the purpose of describing particular embodiments only and is not intended to be limiting of the present disclosure. As used herein, the singular constitutes "a" and "an" are intended to include the plural constitutes as well, unless the context clearly indicates otherwise. It will be further understood that the terms "comprise", "comprising", "include", and "including" when used in this specification, specify the presence of the stated features, integers, operations, elements, and/or components, but do not preclude the presence or addition of one or more other features, integers, operations, elements, components, and/or portions thereof. As used herein, the term "and/or" includes any and all combinations of one or more of the associated listed items. Expression such as "at least one of" when preceding a list of elements may modify an entirety of list of elements and may not modify the individual elements of the list. In interpretation of numerical values, an error or tolerance therein may occur even when there is no explicit description thereof.

Unless otherwise defined, all terms including technical and scientific terms used herein have the same meaning as commonly understood by one of ordinary skill in the art to which this inventive concept belongs. It will be further understood that terms, such as those defined in commonly used dictionaries, should be interpreted as having a meaning that is consistent with their meaning in the context of the relevant art and will not be interpreted in an idealized or overly formal sense unless expressly so defined herein.

Hereinafter, the base oil comprising the polyol ester of the present disclosure and the refrigerating machine oil composition comprising the same will be described in detail.

### Base oil comprising polyol ester (POE)

A base oil for a refrigerating machine oil composition according to the present disclosure is characterized in that the base oil comprises a polyol ester, wherein the polyol ester may have excellent miscibility with refrigerant having high polarity and a low global warming potential (GWP) among variable refrigerants, and may have a high viscosity to increase wear resistance in the refrigerating machine.

Specifically, the polyol ester of the present disclosure has excellent miscibility with various polar refrigerants with a global warming potential of 0 to 2,500. Especially, the polyol ester of the present disclosure has excellent miscibility with environment-friendly refrigerants with a global warming potential of 0 to 750. For example, the refrigerant may include one or more HFC-based refrigerants selected from the group consisting of R134a, which is frequently used in refrigeration systems, R410A, which is frequently used in air conditioning technology systems, and R32, which is an eco-friendly refrigerant, however, refrigerants considered in the present disclosure is not necessarily limited hereto. For example, the polyol ester of the present disclosure may be used with the HC-based refrigerant and/or the HFO-based refrigerant, in addition to the HFC-based refrigerant.

Specific examples of refrigerants that may be applied in addition to the above listed refrigerants may include R1234yf (HFO-based refrigerant), R454B (mixture of HFC-based refrigerant and HFO-based refrigerant), R513A (mixture of HFC-based refrigerant and HFO-based refrigerant), and the like, however, it is not necessarily limited hereto.

The polyol ester preferably has a floc point of -30°C or lower as measured according to a following measurement method (1). The lower the value of the floc point, the better the miscibility with a target refrigerant.

[Measuring method (1)] The floc point is measured according to ASHRAE STANDARD 86, based on a content of 80 vol% of the refrigerant based on a total of 100 vol% of the polyol ester and the refrigerant.

The polyol ester is required to have the excellent miscibility, and at the same time, have high viscosity required for wear resistance of a compressor of the refrigerating machine. Thus, the polyol ester according to the present disclosure is required to have a kinematic viscosity at 40°C (KV40) of 95 to 105 cSt.

Based on a result of intensive research in order to achieve the above technical requirements, the present inventors have derived the polyol ester synthesized using polyhydric alcohol comprising 5 or more hydroxyl groups; a first fatty acid, which is a linear fatty acid having 4 to 6 carbon atoms; a second fatty acid, which is a branched fatty acid having 4 to 6 carbon atoms; and a third fatty acid, which is a linear or branched fatty acid having 7 to 10 carbon atoms, and the synthesized polyol ester is used as the base oil for the refrigerating machine oil composition.

The polyol ester (POE) is generally prepared by synthesizing a polyhydric alcohol (polyol) and a fatty acid. In this regard, the present disclosure has a purpose to provide the POE which has excellent miscibility with refrigerant having relatively high polarity. Therefore, in order to increase the miscibility with the polar refrigerant, the polyol ester is also required to have a high polarity, and at the same time, is also required to be synthesized with a high viscosity to ensure lubricity and .

Therefore, in accordance with the present disclosure, in order to increase the polarity of the polyol ester as synthesized, preferably, the polyhydric alcohol may comprise five or more hydroxyl groups (-OH), for example, five to ten hydroxyl groups. For example, di-pentaerythritol (di-PE), tri-pentaerythritol (tri-PE), and the like may be used.

Further, in accordance with the present disclosure, the polyol ester is synthesized by mixing three types of fatty acids with each other: the first fatty acid, which is a linear fatty acid having 4 to 6 carbon atoms; the second fatty acid, which is a branched fatty acid having 4 to 6 carbon atoms; and the third fatty acid, which is a linear or branched fatty acid having 7 to 10 carbon atoms.

The fatty acid having 4 to 6 carbon atoms such as the first fatty acid and the second fatty acid may be a fatty acid having a relatively smaller number of carbon atoms and may contribute to increasing the polarity of the polyol ester to ensure miscibility with the polar refrigerant. The fatty acids having 7 to 10 carbon atoms such as the third fatty acid may contribute to ensuring lubricity and high viscosity.

Further, irrespective of the number of carbon atoms (chain length) of the fatty acid, the branched fatty acid may increase the polarity of polyol ester and protect the polyhydric alcohol to increase chemical and hydrolytic stability, compared to the linear fatty acid. However, the branched fatty acid has disadvantages of high cost and high coefficient of friction. Thus, it is preferable to mix the branched fatty acid and the linear fatty acid with each other.

In order to synthesize the polyol ester that the present disclosure requires due to the characteristics of the fatty acids as described above, when a total weight of the first fatty acid, the second fatty acid and the third fatty acid is 100 wt%, a content of a combination of the first fatty acid and the second fatty acid is in a range of 50 to 80 wt%, and a content of the third fatty acid is in a range of 20 to 50 wt% which is lower than or equal to the content of the combination of the first fatty acid and the second fatty acid.

More specifically, when the total weight of the first fatty acid and the second fatty acid is 100 wt%, a content of the first fatty acid may be in a range of 30 to 50 wt%, and a content of the second fatty acid may be in a range of 50 to 70 wt%. Accordingly, all of the properties required in the present disclosure, such as the polarity, high viscosity, lubricity, abrasion resistance and chemical stability, may be achieved. As described above, the content of the first fatty acid is lower than or equal to that of the second fatty acid, and the content may be adjusted according to the specific type of the fatty acid.

### Refrigerating machine oil composition

The refrigerating machine oil composition of the present disclosure is prepared by mixing an additive with the base oil containing the polyol ester. For example, the additive may further include at least one selected from the group consisting of a corrosion inhibitor and an acid scavenger, and may further include an additive such as a wear resistance enhancer, or an antioxidant, etc.

The refrigerating machine oil composition according to the present disclosure has a kinematic viscosity at 40°C (KV40) of 70 to 90 cSt, and has a total acid number (TAN) of 0.010 to 0.100 mgKOH/g. In this regard, the total acid number refers to a total acid value, and means an acid value measured according to ASTM D664 Standard Test Method for Acid Number of Petroleum Products by Potentiometric Titration .

When the additive is mixed with the base oil containing the polyol ester, the viscosity of the prepared refrigerating machine oil composition may be somewhat lowered. However, the present disclosure aims to prepare the refrigerating machine oil composition having high viscosity and sufficient lubricity, at the same time. From this point of view, the kinematic viscosity at 40°C (KV40) of the base oil containing the polyol ester according to the present disclosure is in a range of 95 to 105 cSt.

In the refrigerating machine oil composition of the present disclosure, the corrosion inhibitor plays a role in preventing degradation of the refrigerating machine oil and corrosion of the expansion valve. However, when the corrosion inhibitor is added in an excessive amount, there may be a problem in that an initial total acid number (TAN) of the refrigerating machine oil composition becomes excessively high. From this point of view, when the total weight of the refrigerating machine oil composition is 100wt%, a content of the corrosion inhibitor is in a range of 0.03 to 0.10wt%, and more preferably, in a range of 0.03 to 0.05wt%.

In the refrigerating machine oil composition of the present disclosure, the acid scavenger may trap acids resulting from decomposition of the refrigerant such as hydrofluoric acid, thereby increasing operational stability of the refrigerating machine. When the acid scavenger is added in an excessive amount, the total acid number (TAN) of the refrigerating machine oil composition may increase after aging the refrigerating machine oil composition. Thus, when the total weight of the refrigerating machine oil is 100wt%, a content of the acid scavenger is in a range of 0.50 to 3.00wt%, and more preferably, in a range of 1.00wt% to 2.00wt%.

Those commonly used in the art may be used as the corrosion inhibitor. For example, a thiazole-based compound, a triazole-based compound, or a thiadiazole-based compound may be used as the corrosion inhibitor. For example, the triazole-based compound may include a benzotriazole-based compound containing a benzotriazole group in which the compound contains 3 to 12 carbon atoms, preferably, 6 to 10 carbon atoms, excluding the carbon atoms in the benzotriazole group. The present disclosure is not necessarily limited thereto. Specific examples of the compound may include N,N-bis(alkyl)-AR-methyl-1H-benzotriazole-1-methanamine (CAS No. 94270-86-7) or the like.

The acid scavenger may be used generally used in the art. For example, an epoxy-based compound, a carbodiimide compound, a glycidyl ether-based compound, a terpene-based compound, and the like may be used as the acid scavenger. For example, the acid scavenger may include a glycidyl ether-based compound, specifically, triglycidyl ether, diglycidyl ether, glycidyl ether, lauryl glycidyl ether, or the like. However, the kinds of the acid scavenger used in the present disclosure is not necessarily limited hereto.

The refrigerating machine oil composition according to the present disclosure may satisfy a following condition (A):
$1 {\left(TAN\right)}_{f} - {\left(TAN\right)}_{i} 1 \leq 0.03$

The (TAN)ᵢ means a TAN value measured immediately after the preparation of the refrigerating machine oil composition, and the (TAN)_{f} means a TAN value measured after aging of the refrigerating machine oil composition according to ASHRAE STANDARD 97.

The refrigerating machine oil composition may further contain one or more additives such as the antioxidant and the wear resistance enhancer in addition to the corrosion inhibitor and the acid scavenger. However, the present disclosure is not necessarily limited thereto as long as the purpose of the present disclosure may be achieved.

The refrigerating machine oil composition according to the present disclosure may be applied to a typical refrigerating machine in which the above-described refrigerant is used. A ratio of a content of the refrigerant and a content of the composition may be adjusted according to a type and an operating condition of the refrigerating machine.

According to one embodiment, the refrigerating machine oil composition according to the present disclosure may be preferably used, for example, in an air conditioner, a refrigerator, or an air conditioner of an enclosed car. Further, the refrigerating machine oil composition according to the present disclosure may be preferably used for a dehumidifier, a hot water heater, a freezer, a refrigeration and freezing warehouse, a vending machine, a showcase, a cooling device of a chemical plant, and the like. Further, the refrigerating machine oil composition according to the present disclosure may also be preferably used in a cooling device having a centrifugal compressor.

Hereinafter, the present disclosure will be described in more detail based on Examples and Experimental Examples. However, the following Examples and Experimental Examples are merely examples of the present disclosure, and the present disclosure is not limited to the following Examples and Experimental Example.

### <Present Example 1 and Comparative Examples 1 to 4>

Polyol ester of each of Present Example 1 and Comparative Examples 1 to 4 was synthesized using polyhydric alcohol and fatty acids according to Table 1 below.

The KV40 kinematic viscosity of the synthesized polyol ester was measured. The synthesized polyol ester and the refrigerant were mixed with each other in a volume ratio of 2: 8 to prepare a mixture. Then, the floc point of the mixture was measured according to ASHRAE STANDARD 86. The measurement results are shown in a following Table 1.

Further, the polyol ester according to Present Example 1 was mixed with each of various refrigerants listed in Table 2 below, and then the floc point of each mixture was measured. It was determined that the excellent miscibility with the refrigerant as required in the present disclosure was satisfied when the floc point was -30°C or lower. It was interpreted that the lower the floc point value, the higher the miscibility with the refrigerant.

**Table 1**

| | | Present Example 1 | Comparative Example 1 | Comparative Example 2 | Comparative Example 3 | Comparative Example 4 |
|---|---|---|---|---|---|---|
| Polyhydric alcohol | | di-PE | PE | di-PE | di-PE | di-PE |
| Fatty acid (wt%) | iso butanoic acid | 37 | 19 | | 18 | 22 |
| | normal butanoic acid | 22 | | | 22 | 26 |
| | normal valeric acid | | | 77 | | |
| | 2-ethyl hexanoic acid | 41 | | | 60 | 52 |
| | iso nonanoic acid | | 81 | 23 | | |

| **Experimental Example** | | | | | | |
|---|---|---|---|---|---|---|
| KV40 (cSt) | | 97.91 | 68.41 | 68.68 | 108.0 | 102.1 |
| Floc point (°C) (R32) | | -35.7 | -10.7 | -9.6 | -21.7 | -18.1 |

**Table 2**

| | **Present Example 1** |
|---|---|
| Floc point (°C) (R32) | -35.7 |
| Floc point (°C) (R410A) | -60.4 |
| Floc point (°C) (R134a) | -59.9 |
| Floc point (°C) (R1234yf) | -56.6 |
| Floc point (°C) (R454B) | -51.6 |
| Floc point (°C) (R513A) | -56.4 |

### < Present Examples A to B and Comparative Examples A to C>

A refrigerating machine oil composition was prepared by mixing a corrosion inhibitor and an acid scavenger with the polyol ester as prepared in Present Example 1 as described above. Specifically, the refrigerating machine oil composition of each of Present Examples A to B and Comparative Examples A to C was prepared by mixing different types and contents of the corrosion inhibitor and the acid scavenger as described in Table 3 below with the polyol ester as prepared in Present Example 1 as described above.

The initial KV40 and initial TAN values of the prepared refrigerating machine oil compositions (New Oil) were measured. Next, the KV40 and TAN values of the refrigerating machine oil compositions after aging (aged oil) were measured according to ASHRAE STANDARD 97 under the condition of an environment-friendly R32 refrigerant environment. Change in the TAN value before and after the aging was calculated and shown in Table 3 below.

In Table 3 below, a semi-finished product was prepared by mixing the polyol ester prepared in Present Example 1 with the antioxidant and the wear resistance enhancer at the same weight ratio. In Table 3 below, the corrosion inhibitor was N,N-bis(2-ethylhexyl)-AR-methyl-1H-benzotriazole-1-methanamine. 'acid scavenger 1' was lauryl glycidyl ether, 'acid scavenger 2' was butyl glycidyl ether, and 'acid scavenger 3' was trimethylolpropane triglycidyl ether.

**Table 3**

| **Used together with refrigerant R32** | | **Present Example A** | **Present Example B** | **Comparative Example A** | **Comparative Example B** | **Comparative Example C** |
|---|---|---|---|---|---|---|
| Semi-finished product (wt%) | | 97.97 | 97.97 | 99.00 | 98.00 | 99.00 |
| Corrosion inhibitor (wt%) | | 0.03 | 0.03 | | | |
| Acid scavenger | acid scavenger 1 (wt%) | 2.00 | 1.00 | 1.00 | 2.00 | |
| | acid scavenger 2 (wt%) | | 1.00 | | | |
| | acid scavenger 3 (wt%) | | | | | 1.00 |
| Total | | 100.00 | 100.00 | 100.00 | 100.00 | 100.00 |

| **Experimental Example** | | | | | | |
|---|---|---|---|---|---|---|
| New Oil | KV40 (cSt) | 83.15 | 86.86 | 88.88 | 83.36 | 92.60 |
| | TAN (mgKOH/g) | 0.056 | 0.046 | 0.008 | 0.016 | 0.009 |
| Aged Oil | TAN (mgKOH/g) | 0.047 | 0.049 | 0.065 | 0.058 | 0.064 |
| | TAN Change (mgKOH/g) | -0.009 | +0.003 | +0.057 | +0.042 | +0.055 |

As may be seen from Table 3 above, the refrigerating machine oil composition of each of Present Examples A to B as prepared by mixing the polyol ester prepared in Present Example 1 with the antioxidant and the wear resistance enhancer at the same weight ratio according to the present disclosure exhibits the kinematic viscosity and total acid number (TAN) values as desired in the present disclosure, and has excellent chemical stability due to small change in the total acid number even after the aging. This is not the case in the refrigerating machine oil compositions of Comparative Examples A to C.

## Claims

1. A refrigerating machine oil composition comprising:
a base oil comprising polyol ester,
wherein the polyol ester is synthesized using:
a polyhydric alcohol containing 5 or more hydroxyl groups;
a first fatty acid as a linear fatty acid having 4 to 6 carbon atoms;
a second fatty acid as a branched fatty acid having 4 to 6 carbon atoms; and
a third fatty acid as a linear or branched fatty acid having 7 to 10 carbon atoms,
wherein in synthesizing the polyol ester, a sum of a content of the first fatty acid and a content of the second fatty acid is in a range of 50 to 80 wt%, and a content of the third fatty acid is in a range of 20 to 50 wt%, based on 100 wt% of a total weight of the first fatty acid, the second fatty acid, and the third fatty acid,
wherein the polyol ester has a kinematic viscosity at 40°C (KV40) in a range of 95 to 105 cSt,
wherein the refrigerating machine oil further comprises at least one additive selected from a group consisting of a corrosion inhibitor and an acid scavenger, whereby both a corrosion inhibitor and an acid scavenger are present,
wherein the refrigerating machine oil composition has a kinematic viscosity at 40°C (KV40) in a range of 70 to 90 cSt,
wherein a total acid number (TAN) of the refrigerating machine oil composition is in a range of 0.010 to 0.100 mgKOH/g,
wherein when a total weight of the refrigerating machine oil composition is 100 wt%, a content of the corrosion inhibitor is in a range of 0.03 to 0.10 wt%, and a content of the acid scavenger is in a range of 0.50 to 3.00 wt%,
wherein the polyol ester has a floc point of -30°C or lower as measured according to following measurement method (1):
[Measuring method (1)] The floc point is measured according to ASHRAE STANDARD 86, based on a content of 80 vol% of a refrigerant used with the polyol ester and having a global warming potential (GWP) of 0 to 2,500, based on a total of 100 vol% of the polyol ester and the refrigerant,
wherein the refrigerating machine oil composition satisfies a following condition (A): $1 {\left(TAN\right)}_{f} - {\left(TAN\right)}_{i} 1 \leq 0.03$
where (TAN)ᵢ means a TAN value measured immediately after preparation of the refrigerating machine oil composition, and (TAN)_{f} means a TAN value measured after aging of the refrigerating machine oil composition according to ASHRAE STANDARD 97.

2. The refrigerating machine oil composition of claim 1, wherein the refrigerant includes at least one selected from a group consisting of R32, R410A, R134a, R1234yf, R454B and R513A.

3. The refrigerating machine oil composition of claim 1 wherein when a total weight of the first fatty acid and the second fatty acid is 100 wt%, a content of the first fatty acid is in a range of 30 to 50 wt%, and a content of the second fatty acid is in a range of 50 to 70 wt%.

4. The refrigerating machine oil composition of claim 1, wherein the polyhydric alcohol includes dipentaerythritol.

5. The refrigerating machine oil composition of claim 1, wherein the corrosion inhibitor includes a benzotriazole-based compound.

6. The refrigerating machine oil composition of claim 1, wherein the acid scavenger includes a glycidyl ether-based compound.

7. The refrigerating machine oil composition of claim 4, further comprising at least one additive selected from a group consisting of an antioxidant and a wear resistance enhancer.

8. Use of the refrigerating machine oil composition of claim 1 in at least one selected from a group consisting of an air conditioner, a refrigerator, and an air conditioner for a vehicle.

## Patentansprüche

1. Kühlmaschinenölzusammensetzung, umfassend:
ein Basisöl, umfassend Polyolester,
wobei der Polyolester unter Verwendung von Folgendem synthetisiert wird:
einem mehrwertigen Alkohol mit 5 oder mehr Hydroxylgruppen;
einer ersten Fettsäure als eine lineare Fettsäure, die 4 bis 6 Kohlenstoffatome aufweist;
einer zweiten Fettsäure als eine verzweigte Fettsäure, die 4 bis 6 Kohlenstoffatome aufweist; und
einer dritten Fettsäure als eine lineare oder verzweigte Fettsäure, die 7 bis 10 Kohlenstoffatome aufweist,
wobei beim Synthetisieren des Polyolesters eine Summe eines Gehalts der ersten Fettsäure und eines Gehalts der zweiten Fettsäure im Bereich von 50 bis 80 Gew.-% liegt und ein Gehalt der dritten Fettsäure im Bereich von 20 bis 50 Gew.-% liegt, basierend auf 100 Gew.-% eines Gesamtgewichts der ersten Fettsäure, der zweiten Fettsäure und der dritten Fettsäure,
wobei der Polyolester bei 40 °C (KV40) eine kinematische Viskosität im Bereich von 95 bis 105 cSt aufweist,
wobei das Kühlmaschinenöl ferner mindestens ein Additiv umfasst, das aus einer Gruppe ausgewählt ist, die aus einem Korrosionsinhibitor und einem Säurefänger besteht, wobei sowohl ein Korrosionsinhibitor als auch ein Säurefänger vorhanden sind, wobei die Kühlmaschinenölzusammensetzung bei 40 °C (KV40) eine kinematische Viskosität in einem Bereich von 70 bis 90 cSt aufweist,
wobei eine Gesamtsäurezahl (TAN) der Kühlmaschinenölzusammensetzung im Bereich von 0,010 bis 0,100 mgKOH/g liegt,
wobei, wenn ein Gesamtgewicht der Kühlmaschinenölzusammensetzung 100 Gew.-% beträgt, ein Gehalt des Korrosionsinhibitors im Bereich von 0,03 bis 0,10 Gew.-% liegt und ein Gehalt des Säurefängers im Bereich von 0,50 bis 3,00 Gew.-% liegt,
wobei der Polyolester einen Flockungspunkt von -30 °C oder weniger aufweist, gemessen gemäß dem folgenden Messverfahren (1):
[Messverfahren (1)] Der Flockungspunkt wird gemäß dem ASHRAE STANDARD 86 gemessen, basierend auf einem Gehalt von 80 Vol.-% eines Kühlmittels, das mit dem Polyolester verwendet wird und das ein Treibhauspotenzial (GWP) von 0 bis 2.500 aufweist, basierend auf insgesamt 100 Vol.-% des Polyolesters und des Kühlmittels,
wobei die Kühlmaschinenölzusammensetzung eine folgende Bedingung (A) erfüllt: $1 {\left(TAN\right)}_{f} - {\left(TAN\right)}_{i} 1 \leq 0,03$
wobei (TAN)ᵢ einen TAN-Wert, der unmittelbar nach Herstellung der Kühlmaschinenölzusammensetzung gemessen wird, bedeutet und (TAN)_{f} einen TAN-Wert, der nach Altern der Kühlmaschinenölzusammensetzung gemäß ASHRAE STANDARD 97 gemessen wird, bedeutet.

2. Kühlmaschinenölzusammensetzung nach Anspruch 1, wobei das Kühlmittel mindestens eines beinhaltet, das aus einer Gruppe ausgewählt wurde, die aus R32, R410A, R134a, R1234yf, R454B und R513A besteht.

3. Kühlmaschinenölzusammensetzung nach Anspruch 1, wobei, wenn ein Gesamtgewicht der ersten Fettsäure und der zweiten Fettsäure 100 Gew.-% beträgt, ein Gehalt der ersten Fettsäure im Bereich von 30 bis 50 Gew.-% liegt und ein Gehalt der zweiten Fettsäure im Bereich von 50 bis 70 Gew.-% liegt.

4. Kühlmaschinenölzusammensetzung nach Anspruch 1, wobei der mehrwertige Alkohol Dipentaerythrit beinhaltet.

5. Kühlmaschinenölzusammensetzung nach Anspruch 1, wobei der Korrosionsinhibitor eine auf Benzotriazol basierende Verbindung beinhaltet.

6. Kühlmaschinenölzusammensetzung nach Anspruch 1, wobei der Säurefänger eine auf Glycidylether basierende Verbindung beinhaltet.

7. Kühlmaschinenölzusammensetzung nach Anspruch 4, ferner umfassend mindestens ein Additiv, das aus einer Gruppe ausgewählt ist, die aus einem Antioxidationsmittel und einem Mittel zur Verbesserung der Verschleißfestigkeit besteht.

8. Verwendung der Kühlmaschinenölzusammensetzung nach Anspruch 1 in mindestens einem, das aus einer Gruppe ausgewählt ist, die aus einer Klimaanlage, einem Kühlschrank und einer Klimaanlage für ein Fahrzeug besteht.

## Revendications

1. Composition d'huile pour machine frigorifique comprenant
une huile de base comprenant un ester de polyol,
dans laquelle l'ester de polyol est synthétisé en utilisant :
un alcool polyhydrique contenant 5 groupes hydroxyles ou plus ;
un premier acide gras sous forme d'acide gras linéaire ayant 4 à 6 atomes de carbone ;
un deuxième acide gras sous forme d'acide gras ramifié ayant 4 à 6 atomes de carbone ; et
un troisième acide gras sous forme d'acide gras linéaire ou ramifié ayant 7 à 10 atomes de carbone,
dans lequel, lors de la synthèse de l'ester de polyol, la somme de la teneur du premier acide gras et de la teneur du deuxième acide gras est comprise entre 50 et 80 % en poids, et la teneur du troisième acide gras est comprise entre 20 et 50 % en poids, sur la base de 100 % en poids du poids total du premier acide gras, du deuxième acide gras et du troisième acide gras,
dans lequel l'ester de polyol a une viscosité cinématique à 40°C (KV40) dans une plage de 95 à 105 cSt,
dans laquelle l'huile pour machine frigorifique comprend en outre au moins un additif choisi dans un groupe constitué d'un inhibiteur de corrosion et d'un capteur d'acide, un inhibiteur de corrosion et un capteur d'acide étant tous deux présents,
dans laquelle la composition d'huile pour machine frigorifique a une viscosité cinématique à 40°C (KV40) dans une plage de 70 à 90 cSt,
dans laquelle l'indice d'acide total (TAN) de la composition d'huile pour machine frigorifique est compris entre 0,010 et 0,100 mgKOH/g,
dans laquelle lorsque le poids total de la composition d'huile pour machine frigorifique est de 100 % en poids, la teneur en inhibiteur de corrosion est comprise entre 0,03 et 0,10 % en poids et la teneur en capteur d'acide est comprise entre 0,50 et 3,00 % en poids,
dans laquelle l'ester de polyol a un point de floculation de - 30 °C ou moins tel que mesuré selon le procédé de mesure suivant (1) :
[Procédé de mesure (1)] Le point de floculation est mesuré selon la norme ASHRAE 86, sur la base d'une teneur de 80 % en volume d'un réfrigérant utilisé avec l'ester de polyol et ayant un potentiel de réchauffement global (PRG) de 0 à 2 500, sur la base d'un total de 100 % en volume de l'ester de polyol et du réfrigérant,
dans laquelle la composition d'huile pour machine frigorifique satisfait à la condition suivante (A) : $1 {\left(TAN\right)}_{f} - {\left(TAN\right)}_{i} 1 \leq 0,03$
où (TAN)ᵢ signifie une valeur TAN mesurée immédiatement après la préparation de la composition d'huile pour machine frigorifique, et (TAN)_{f} signifie une valeur TAN mesurée après vieillissement de la composition d'huile pour machine frigorifique conformément à la norme ASHRAE 97.

2. Composition d'huile pour machine frigorifique selon la revendication 1, dans laquelle le réfrigérant comprend au moins un élément choisi dans un groupe constitué de R32, R410A, R134a, R1234yf, R454B et R513A.

3. Composition d'huile pour machine frigorifique selon la revendication 1, dans laquelle, lorsque le poids total du premier acide gras et du deuxième acide gras est de 100 % en poids, la teneur du premier acide gras est comprise entre 30 et 50 % en poids et la teneur du deuxième acide gras est comprise entre 50 et 70 % en poids .

4. Composition d'huile pour machine frigorifique selon la revendication 1, dans laquelle l'alcool polyhydrique comprend du dipentaérythritol.

5. Composition d'huile pour machine frigorifique selon la revendication 1, dans laquelle l'inhibiteur de corrosion comprend un composé à base de benzotriazole.

6. Composition d'huile pour machine frigorifique selon la revendication 1, dans laquelle le capteur d'acide comprend un composé à base d'éther glycidylique.

7. Composition d'huile pour machine frigorifique selon la revendication 4, comprenant en outre au moins un additif choisi dans un groupe constitué d'un antioxydant et d'un agent améliorant la résistance à l'usure.

8. Utilisation de la composition d'huile pour machine frigorifique selon la revendication 1 dans au moins un appareil choisi dans un groupe constitué d'un climatiseur, d'un réfrigérateur et d'un climatiseur pour véhicule.
